

# UNITED STATES PATENT OFFICE.

BERTRAND S. SUMMERS, OF PORT HURON, MICHIGAN, ASSIGNOR TO SUMMERS LINEN COMPANY, A CORPORATION OF MAINE.

## PREPARING BAST FIBER, SUCH AS FLAX OR HEMP, FOR SPINNING.

1,127,811.

Specification of Letters Patent.

Patented Feb. 2, 1915.

No Drawing.

Application filed June 12, 1911. Serial No. 332,570.

To all whom it may concern:

Be it known that I, BERTRAND S. SUMMERS, a citizen of the United States, residing at Port Huron, in the county of St. Clair and State of Michigan, have invented certain new and useful Improvements in the Art of Preparing Bast Fiber, Such as Flax or Hemp, for Spinning, of which the following is a specification.

Such fibers contain certain carbo-hydrates known as pectoses and similar substances, the presence of which in their natural state interferes with the spinning qualities of the fibers, and it is necessary in order to put the latter in proper condition for spinning to subject them to treatment by which the objectionable matter is either removed or so altered as to be no longer detrimental, the precise character of the changes effected not being fully understood. The more usual treatment for this purpose consists in what is known as a retting process which as generally carried out hitherto and known as the natural retting process consists in either submitting the raw material to the natural elements on grassy ground or in immersing it in water for a considerable period under certain definite conditions. As a result of this treatment, the objectionable matter becomes partially dissolved and softened or otherwise altered so that it may be readily washed or otherwise removed to a greater or less extent leaving the fiber in proper condition for spinning with substantially its original strength preserved.

My invention relates to a substitute for this so-called natural treatment and is especially adapted to flax fibers though it will be readily apparent from what follows that it is also applicable with slight, or no modification to a variety of other fibers.

My invention is based upon the discovery that by introducing into the fibers nitrogenous material of a certain character under suitable conditions it is possible to reproduce the effect of natural retting on fiber, securing a result equal, if not superior, thereto and very materially reducing the time required for treatment. I prefer to use as the albuminoid or nitrogenous substance, milk casein which when decomposed either by a suitable re-agent or by putrefaction yields amido acid or fatty substances, such as glvcocol, leucin, et cetera. These

products of decomposition of nitrogenous matters are especially effective in producing the desired solvent or other action upon the gummy, pectose and other matters of which it is desired to free the fiber, and at the same time they do not produce the weakening and other ill effects of many or all of the solvents which it has heretofore been proposed to use in place of the natural retting process. I have found also that by my process that essential property of fibers which enters into and affects the spinning of the same known as nature is improved over that obtained by processes hitherto known to me and the dyeing properties of the fiber are also benefited.

The nitrogenous material may be prepared in a variety of ways. Thus, I have found that very good results may be obtained by allowing the albuminoid or other nitrogenous substances to ferment or partially putrefy before employing them in the treatment of fiber, or if preferred I make the solution for treatment of the fiber contain about two per cent. casein and two per cent. sal soda, varying it somewhat according to the fiber to be treated, and use enough water to thoroughly cover and permeate the fibrous mass. Preferably for a good high grade fiber I subject the fiber to a number of treatments in such solutions and afterward the fibrous mass is thoroughly washed out in plain water and carefully dried. I may also employ other alkalis instead of sal soda, such as for example caustic soda, although the strength is not quite as good as when the preferred re-agent is used, a very good grade of fiber, however, resulting. For the best effect, however, the fiber previous to its treatment with albuminoid or nitrogenous substances is subjected to an alkali treatment, for which purpose sodium carbonate or sal soda is satisfactory. When this method is adopted I make a hot solution of the alkali, which in the case of sal soda may be saturated or of a less strength, and boil the fiber therein for about one hour with or without the addition of a small percentage of casein to the solution. After the alkali treatment, I remove the fiber, drain it and introduce it into a solution of casein dissolved in a small amount of sal soda. For this purpose the proportions above specified, i. e. 2% casein and 2% sal soda, have been found effective though they

may be widely varied, as above stated, according to the fiber being treated.

While I have described the use of casein as the principal re-agent in my process, it will be obvious that a great variety of other nitrogenous matters of animal origin are available for the purpose and I am not limited, therefore, to the employment of casein. Again I have described boiling as a suitable method of securing the desired penetration of the nitrogenous matters within the mass of fibers, though this is not essential, but, on the other hand very satisfactory results may be obtained by simply soaking the fiber in the re-agent, the reaction in this case being slower, and the preliminary treatment with alkali, as heretofore stated, may be widely varied or omitted altogether without departing from the spirit of my invention.

I claim:

1. The herein described process of preparing fibers for spinning which consists in subjecting them to decomposed casein.
2. The herein described process of preparing vegetable fibers for spinning which consists in treating them with an alkali and then subjecting them to the action of a solution of a nitrogenous animal product.
3. The herein described process of preparing and retting vegetable fibers for spinning which consists in subjecting them to the action of an alkali and animal decomposition products.

BERTRAND S. SUMMERS.

Witnesses:

G. J. SMITH,  
C. D. BEARD.